

Patented Oct. 10, 1950

2,525,700

# UNITED STATES PATENT OFFICE

2,525,700

## CARBURIZING

George K. Manning, Philip C. Rosenthal, and  
George P. Krumlauf, Columbus, Ohio, assignors  
to Battelle Memorial Institute, Columbus, Ohio,  
a corporation of Ohio

No Drawing. Application December 3, 1943,  
Serial No. 512,834

1 Claim. (Cl. 148—30)

1

This invention relates to the art of carburizing. It is particularly concerned with a new and improved carburizing compound and method whereby the carbon concentration, and particularly the maximum carbon concentration, of the carburized case may be controlled.

In commercial carburizing it is often desirable to control not only the rate and depth of carbon penetration but also the maximum carbon concentration in the carburized material. The depth of penetration usually can be rather easily controlled by varying the time and temperature of the carburizing cycle. The rate of penetration is also somewhat dependent upon the time and temperature of the carburizing cycle and, in addition, can be affected somewhat by the addition of certain "energizers" to the carburizing medium. The maximum carbon concentration in the carburized case is, however, not susceptible to such ready control.

Solid commercial carburizers commonly result in cases having maximum carbon concentrations ranging upward from 0.90 per cent carbon. In many commercial applications such high carbon concentrations, in excess of 0.90 per cent, are regarded as an advantage. This is particularly true when high abrasion resistance is required.

On the other hand, in numerous applications abrasion resistance is of little or no importance and high surface hardness is the principal requirement. The hardness of a carburized case does not increase proportionately as the maximum carbon content increases in the higher ranges. In fact, as is discussed by Burns, Moore, and Archer, Transactions of American Society for Metals, volume XXVI, 1938, page 14, the maximum hardness curve levels off at about 0.50 per cent carbon and further increases in this element do not increase the hardness appreciably. However, although the hardness does not increase, the ductility and the toughness of the case continue to decrease as the carbon content is increased. Therefore, in order to obtain a case with the best combination of hardness and toughness, a maximum carbon concentration substantially less than 0.90 per cent, and in many instances preferably about 0.50 per cent, is often desired.

The best combination of hardness and toughness is desired in many applications. As typical examples, gears, camshafts, pinions, bearings, and face-hardened armor plate may be mentioned. In the production of face-hardened armor, for example, considerable difficulty is often encountered during the straightening operation. The low ductility and toughness of the case structure, resulting from the relatively high carbon content of the case, causes considerable loss in production because of breakage. For this reason it is extremely important to restrict the maximum carbon content of the case of the face-hardened armor to the lowest level commensurate with satisfactory hardness,

2

thereby obtaining the maximum practical ductility and hardness in the case. In this particular application, a further advantage is obtained inasmuch as increased case ductility tends to improve the ballistic resistance of the armor.

One way that these relatively low carbon cases may be obtained is by a diffusion period following the carburizing period. In gas carburizing, this can be accomplished without too much difficulty by proportioning the carburizing and inert gases of the mixture so that the carburizing and diffusion steps either occur simultaneously or follow each other. The main disadvantage in this procedure is the additional furnace time required. On the other hand, in pack carburizing using a solid compound, the problem is not so readily solved and two separate cycles are required. The process becomes quite costly, therefore, both because of the double handling and because of the additional furnace time required.

20 A further method of restricting the maximum carbon content of the case has been proposed. It has been suggested that the addition of ferrosilicon, or of certain other silicon-containing materials, to a standard commercial carburizer is effective in limiting the maximum carbon content of the case produced in a single carburizing treatment. The addition of approximately 20 per cent of finely ground ferrosilicon to the carburizing compound tends to eliminate from the case the hypereutectoid zones, that is those zones containing in excess of about 0.85 to 0.95 per cent carbon depending upon the composition of the base material. With this treatment, however, a substantial portion of the case is of eutectoid composition, containing an average of from about 0.85 to 0.95 per cent carbon in most instances. Although such cases may be used for certain applications, for example, idler shafts and other surfaces requiring high abrasion resistance; there are numerous other applications, such as roller bearings, piston pins, transmission gears, camshafts, machine gun ejector parts, and armor plate, where it may be particularly desirable to limit the maximum carbon content of the case to the hypoeutectoid range, that is, containing less than about 0.85 to 0.95 per cent carbon. As has been mentioned previously, in some instances particular advantages may be gained by restricting the carbon content of the case to a maximum value as low as 0.50 per cent or even lower.

It is therefore one object of our invention to provide an improved method for regulating the carbon concentration within the case of carburized material.

55 Another object of this invention is to provide a carburizing compound that is capable of yielding a case having an essentially hypoeutectoid structure.

60 A further object of our invention is to develop a process for limiting the maximum carbon concentration in a carburized case to a value less than about 0.85 per cent and preferably to any

desired carbon content within the range of from about 0.45 to about 0.75 per cent.

Yet a further object of this invention is to regulate the carbon concentration at or near the surface of carburized material in a predictable manner without resorting to a diffusion treatment.

Still another object of our invention is to provide an improved method for the production of face-hardened armor having a superior combination of hardness and toughness or ductility in the carburized case.

Other and further objects of this invention will be apparent from the following description and the appended claims.

We have discovered that the maximum carbon content of a carburized case may be appreciably lowered to within the hypoeutectoid range without double handling and in less time than is required for both a carburizing and diffusion treatment by the use of a carburizing compound composed essentially of a varying amount of a metallic chloride, hereinafter referred to as "chloride," and a silicon-containing material and a carbonaceous base. With a carburizing compound of this type, a case with a low maximum carbon content can be obtained and that maximum can be controlled and predetermined by proper choice of the amount and kind of chlorides and silicon-containing materials used with the carburizing compound.

In general, we have found a total chloride addition of from about 0.5 to about 15 per cent is effective; however, we prefer to add from about 2 to about 8 per cent. Although additions in excess of 15 per cent may be used, the additional benefits obtained are not commensurate with the increased costs. As previously mentioned, the inhibiting effect obtained depends upon the nature of the chloride as well as upon the quantity and nature of the silicon-bearing material employed. By varying the chloride content within the limits mentioned, we have found it possible to obtain maximum carbon concentrations ranging from a value of about 0.40 per cent up to that normally developed by the use of the untreated carburizer.

The addition of from about 2 to about 25 per cent of silicon as a silicon-containing material is desirable; however, we prefer to add from

about 5 to about 15 per cent of silicon as a silicon-bearing agent. Additions in excess of 25 per cent may be made; however, the dilution effect tends to become excessive when too much is added. The particle size of the silicon-containing material has an effect upon the results produced. In general, the effectiveness of the silicon addition increases as the particle size of the material is decreased. For most purposes, 10 the best results are obtained in the use of ferrosilicon and calcium silicide when the material is finer than 80-mesh; with silicon carbide, we prefer to use a particle size at least 100-mesh or finer.

15 The desirable results obtained by means of the combined additions of chlorides and silicon-bearing materials to a commercial carburizing compound are illustrated by the following data. For these tests, a commercial carburizer, composed 20 essentially of coke and charcoal along with 1.1% sodium, 2.6% calcium, and 7.0% barium in the form of their carbonates was used on the carbonaceous base. This carburizer gives a relatively low carbon content by itself. Additions of 25 chlorides and silicon-containing materials, in accordance with our invention, were added to this base. A carburizing cycle consisting of holding for 24 hours at 1700° F. was used. The carbon concentrations were determined by analyzing 30 turnings from successive layers. The first layer from each sample was 0.002-inch thick; the second, 0.003 inch thick; and the next three layers, 0.005 inch thick. Eight additional layers, each 0.010 inch thick, were then turned from the 35 specimen. The maximum carbon concentration was usually found in the 0.002 inch thick layer.

Table I shows the effect of the addition of various amounts of several different chlorides on the maximum carbon content of the carburized case. 40 As is shown by this table, the maximum carbon content of the case decreases progressively as increasing amounts of nickel chloride, chromium chloride, or combinations of the two are added to a carburizing compound containing, in addition, a silicon-containing material. For example, the addition of 8 per cent nickel chloride and 15 per cent silicon carbide to a carburizer that normally gives a maximum carbon content of 0.95 per cent, results in a case having 45 a maximum carbon content of 0.43 per cent.

TABLE I  
Effect of various chloride additions on maximum carbon content of the carburized case

| Specimen No. | Composition of Carburizing Compound, Per Cent |         |                     |                       | Maximum Carbon Content |
|--------------|-----------------------------------------------|---------|---------------------|-----------------------|------------------------|
|              | Chlorides                                     | Silicon | Silicon Added As—   | Commercial Carburizer |                        |
|              |                                               |         |                     | Per cent              |                        |
| 1.           |                                               |         |                     |                       |                        |
| 17           | 1-NiCl <sub>2</sub>                           | 10      | 15-SiC              |                       | 100 0.95               |
| 18           | 2-NiCl <sub>2</sub>                           | 10      | do                  |                       | 84 0.78                |
| 2            | 4-NiCl <sub>2</sub>                           | 10      | do                  |                       | 83 0.73                |
| 19           | 8-NiCl <sub>2</sub>                           | 10      | do                  |                       | 81 0.53                |
| 20           | 1-CrCl <sub>3</sub>                           | 10      | do                  |                       | 77 0.43                |
| 21           | 2-CrCl <sub>3</sub>                           | 10      | do                  |                       | 84 0.86                |
| 3            | 4-CrCl <sub>3</sub>                           | 10      | do                  |                       | 83 0.81                |
| 22           | 8-CrCl <sub>3</sub>                           | 10      | do                  |                       | 81 0.65                |
| 34           | ½-NiCl <sub>2</sub> , ½-CrCl <sub>3</sub>     | 10      | do                  |                       | 77 0.62                |
| 35           | 1-NiCl <sub>2</sub> , 1-CrCl <sub>3</sub>     | 10      | do                  |                       | 84 0.78                |
| 4            | 2-NiCl <sub>2</sub> , 2-CrCl <sub>3</sub>     | 10      | do                  |                       | 83 0.69                |
| 76           | 2-NaCl                                        | 7       | 14-FeSi             |                       | 81 0.66                |
| 56           | 4-NaCl                                        | 7       | do                  |                       | 82 0.89                |
| 77           | 6-NaCl                                        | 7       | do                  |                       | 80 0.64                |
| 66           | 8-NaCl                                        | 7       | do                  |                       | 78 0.74                |
| 49           | 4-CuCl <sub>2</sub>                           | 10      | 15-SiC              |                       | 81 0.74                |
| 70           | 4-CaCl <sub>2</sub>                           | 10      | 20-SiO <sub>2</sub> |                       | 76 0.62                |

As is also shown by Table I, the addition of 2 or 6 per cent of sodium chloride is more effective than an addition of 4 or 8 per cent of the same material. There is also a tendency toward pitting of the surface of the case when sodium chloride additions of 6 per cent or more are used. This pitting effect is not found when other chlorides are used.

For a given concentration, nickel chloride ranks high in its inhibiting effect while barium chloride, for example, is much less effective. As a general rule, the most effective chlorides are those

5 con-bearing material, act as energizers rather than as inhibitors. The addition of a silicon-containing material, in the absence of a chloride, does effect a slight lowering of the maximum carbon concentration; however, this effect appears to be primarily that of dilution as is indicated by the results obtained from the addition of a relatively inert material such as magnesia. It is clearly evident that the desirable results of our invention are obtained only through the use of a combination of a chloride and a silicon-containing agent.

TABLE II  
Effect of various silicon additions on the maximum carbon content of the carburized case

| Specimen No. | Composition of Carburizing Compound, Per Cent |         |                     |                       | Maximum Carbon Content |
|--------------|-----------------------------------------------|---------|---------------------|-----------------------|------------------------|
|              | Chlorides                                     | Silicon | Silicon Added As—   | Commercial Carburizer |                        |
| 1            |                                               |         |                     |                       | Per cent               |
| 11           | 4-NiCl <sub>2</sub>                           | 1       | 2-SiC               | 100                   | 0.95                   |
| 8            | do                                            | 3.5     | 5-SiC               | 94                    | 0.91                   |
| 7            | do                                            | 7       | 10-SiC              | 91                    | 0.80                   |
| 2            | do                                            | 10      | 15-SiC              | 86                    | 0.61                   |
| 9            | do                                            | 12      | 20-SiC              | 81                    | 0.53                   |
| 10           | do                                            | 21      | 30-SiC              | 76                    | 0.62                   |
| 42           | 2-NiCl <sub>2</sub> , 2-CrCl <sub>3</sub>     | 3.5     | 7-FeSi              | 66                    | 0.47                   |
| 41           | do                                            | 7       | 14-FeSi             | 89                    | 0.82                   |
| 40           | do                                            | 10      | 20-FeSi             | 82                    | 0.54                   |
| 45           | do                                            | 3.3     | 5.5-CaSi            | 76                    | 0.45                   |
| 44           | do                                            | 6.6     | 11-CaSi             | 90.5                  | 0.86                   |
| 43           | do                                            | 10      | 16.5-CaSi           | 85                    | 0.78                   |
| 73           | do                                            | 10      | 20-SiO <sub>2</sub> | 79.5                  | 0.78                   |
| 61           | 4-NaCl                                        | 7       | 7.8-FeSi            | 76                    | 0.74                   |
|              |                                               |         |                     | 88.2                  | 0.84                   |

TABLE III  
Effect of chloride and silicon-containing additions when made singly

| Specimen No. | Composition of Carburizing Compound, Per Cent |         |                   |                       | Maximum Carbon Content |
|--------------|-----------------------------------------------|---------|-------------------|-----------------------|------------------------|
|              | Chlorides                                     | Silicon | Silicon Added As— | Commercial Carburizer |                        |
| 1            |                                               |         |                   |                       | Per cent               |
| 47           | 2-NiCl <sub>2</sub> , 2-CrCl <sub>3</sub>     |         |                   |                       | 100                    |
| 46           |                                               |         |                   |                       | 96                     |
| 65           |                                               |         |                   |                       | 1.12                   |
| 75           |                                               |         |                   |                       | 85                     |
|              |                                               |         |                   |                       | 0.87                   |
|              |                                               |         |                   |                       | 86                     |
|              |                                               |         |                   |                       | 0.85                   |
|              |                                               |         |                   |                       | 1.80                   |
|              |                                               |         |                   |                       | 0.88                   |

<sup>1</sup> Carburizer diluted with 20% MgO.

having a boiling point in excess of the carburizing temperature.

Table II shows the effect of the addition of various chlorides. The maximum carbon content tends to vary progressively with increases in silicon additions. From the data in Tables I and II it is apparent that, for an addition equivalent to 10 per cent of silicon, ferrosilicon is slightly more effective than silicon carbide, while silicon carbide is somewhat more effective than silica or calcium silicide. However, even silica is an effective silicon-bearing addition as is indicated by the fact that the addition of 4 per cent calcium chloride and 20 per cent silica flour reduced the maximum carbon content of the resulting case from 0.95 to 0.62 per cent.

The necessity of adding both a chloride and a silicon-containing material is clearly shown by the data in Table III. It is interesting to note that chloride additions, in the absence of a sili-

55 carbonaceous base, preferably an energized commercial carburizer, is thoroughly mixed with the desired amount of silicon-containing material. The required amount of chloride is then dissolved in a suitable binder, such as molasses water, and the resulting solution added to the dry mixture. The whole is then thoroughly mixed and dried. We have found that, in some instances, a slightly moist compound gives somewhat lower carbon concentrations than does a thoroughly dried compound. However, the results tend to be less reproducible when the moist compound is used, probably because of the difficulty in accurately reproducing the same moisture content.

In the use of the carburizing compound of our invention, any normal carburizing cycle may be used. For most purposes, carburizing temperatures between about 1600° and 1800° F. are in

common use, while a temperature around 1700° F. is usually preferred. Although the time at carburizing temperature affects the depth of the case, it has relatively small effect upon the maximum carbon concentration. For example, specimens carburized in a compound containing 2 per cent nickel chloride, 2 per cent chromium chloride, 15 per cent silicon carbide, and the balance commercial carburizer, for periods of 4, 8, 14, 16, and 24 hours, had cases with maximum carbon concentrations of 0.67, 0.60, 0.68, 0.58, and 0.60 per cent respectively.

It is possible to reuse the mixture by merely replacing that which is consumed and that which is lost by dusting and by drag-out. In one test, the same mixture was reused five times. After each cycle, the compound was passed over a No. 10 screen and the fines discarded. Twenty-five per cent of the weight of the remaining coarse particles was added as fresh mixture after each of the first four cycles and eleven per cent after the fifth cycle. The results indicated a rather abrupt decrease in maximum carbon content between the second and third cycle. Thereafter, no conspicuous change occurred.

The above examples are given merely to illustrate the principles, compositions, and methods of our invention, and it will be understood that variations are possible within the scope of the appended claims.

Unless otherwise specified, all percentages referred to herein will be understood to represent percentages by weight rather than by volume.

From the foregoing description of our invention, it will be apparent that we have provided a novel carburizing agent that is capable of producing, in a single-treatment process, carburized cases having maximum carbon concentrations substantially below those produced by the carburizing processes known heretofore. This highly desirable effect is obtained by the incor-

poration of a combination of one or more chlorides and a silicon-containing material in an essentially standard carburizer. Although neither chlorides nor silicon-containing materials are suitable for the purposes herein disclosed when added alone, the addition of the two in combination results in a marked reduction in the maximum carbon concentration of a case produced by a normal carburizing cycle.

Having thus described our invention, what we claim is:

A carburizing compound having a base composed of an energized carburizing material and containing in addition, about 2 per cent nickel chloride, about 2 per cent chromium chloride, and about 15 per cent silicon carbide.

GEORGE K. MANNING.  
PHILIP C. ROSENTHAL.  
GEORGE P. KRUMLAUF.

#### REFERENCES CITED

The following references are of record in the file of this patent:

#### UNITED STATES PATENTS

|    | Number    | Name          | Date          |
|----|-----------|---------------|---------------|
|    | 787,926   | Lecarme       | Apr. 26, 1905 |
|    | 1,076,453 | Rodman        | Oct. 21, 1913 |
|    | 1,310,918 | Mebane        | July 22, 1919 |
| 30 | 1,593,132 | Nelson        | July 20, 1926 |
|    | 1,921,367 | Mohin         | Aug. 8, 1933  |
|    | 2,149,747 | Redman        | Mar. 7, 1939  |
|    | 2,188,063 | Solakian      | Jan. 23, 1940 |
|    | 2,249,581 | Solakian      | July 15, 1941 |
| 35 | 2,263,906 | Solakian      | Nov. 25, 1941 |
|    | 2,320,872 | Kramer et al. | June 1, 1943  |

#### FOREIGN PATENTS

|    | Number | Country       | Date    |
|----|--------|---------------|---------|
| 40 | 3,586  | Great Britain | of 1893 |
|    | 25,986 | Great Britain | of 1903 |

**Certificate of Correction**

Patent No. 2,525,700

October 10, 1950

**GEORGE K. MANNING ET AL.**

It is hereby certified that error appears in the printed specification of the above numbered patent requiring correction as follows:

Column 5, lines 67 to 69, inclusive, beginning with the syllable "ous" strike out all to and including the word "case" in line 69, and insert the same before "tends" in line 57, same column;

and that the said Letters Patent should be read as corrected above, so that the same may conform to the record of the case in the Patent Office.

Signed and sealed this 16th day of January, A. D. 1951.

[~~SEAL~~]

**THOMAS F. MURPHY,**  
*Assistant Commissioner of Patents.*